



US005576163A

**United States Patent**

[19]

**Anderson et al.**[11] **Patent Number:** **5,576,163**[45] **Date of Patent:** **Nov. 19, 1996**

[54] **IMAGING ELEMENT HAVING A  
PROCESS-SURVIVING  
ELECTRICALLY-CONDUCTIVE LAYER  
WITH POLYESTERIONOMER BINDER**

[75] Inventors: **Charles C. Anderson**, Penfield; **Mario D. DeLaura**, Hamlin, both of N.Y.

[73] Assignee: **Eastman Kodak Company**, Rochester, N.Y.

[21] Appl. No.: **625,118**

[22] Filed: **Apr. 1, 1996**

[51] **Int. Cl.<sup>6</sup>** ..... **G03C 1/89**; B32B 27/06; C08K 3/10; H01B 1/06

[52] **U.S. Cl.** ..... **430/529**; 430/530; 430/626; 252/518; 428/482; 524/408

[58] **Field of Search** ..... 430/527, 529, 430/530, 626; 428/482; 252/518; 524/408

[56] **References Cited**

U.S. PATENT DOCUMENTS

4,203,769 5/1980 Guestaux ..... 430/628  
5,006,451 4/1991 Anderson et al. ..... 430/530

5,096,975 5/1992 Anderson et al. ..... 430/529  
5,198,499 3/1993 Anderson et al. ..... 430/527  
5,203,884 4/1993 Buchanan et al. ..... 51/295  
5,221,598 6/1993 Anderson et al. ..... 430/527  
5,322,761 6/1994 Kausch et al. ..... 430/273  
5,360,706 11/1994 Anderson et al. ..... 430/530  
5,372,985 12/1994 Chang et al. ..... 503/201  
5,407,603 4/1995 Morrison ..... 430/527  
5,424,269 6/1995 Chang et al. ..... 503/227  
5,427,835 6/1995 Morrison et al. ..... 430/527  
5,439,785 8/1995 Boston et al. ..... 430/530  
5,468,498 11/1995 Morrison et al. ..... 524/408

*Primary Examiner*—Richard L. Schilling  
*Attorney, Agent, or Firm*—Alfred P. Lorenzo

[57] **ABSTRACT**

Imaging elements, such as photographic, electrostatographic and thermal imaging elements are comprised of a support, an image-forming layer and an electrically-conductive layer comprised of a vanadium pentoxide colloidal gel, a polyesteronomer binder and a methoxyalkylmelamine. The electrically-conductive layer exhibits electrical conductivity which is both process-surviving and essentially independent of humidity.

**15 Claims, No Drawings**

**IMAGING ELEMENT HAVING A  
PROCESS-SURVIVING  
ELECTRICALLY-CONDUCTIVE LAYER  
WITH POLYESTERIONOMER BINDER**

**FIELD OF THE INVENTION**

This invention relates in general to imaging elements, such as photographic elements, and in particular to imaging elements comprising a support, an image-forming layer and an electrically-conductive layer. More specifically, this invention relates to imaging elements having an electrically-conductive layer whose electrical conductivity is process-surviving and essentially independent of humidity.

**BACKGROUND OF THE INVENTION**

The problem of controlling static charge is well known in the field of photography. Static charging may occur due to various factors in the manufacture, finishing, and use of photographic elements. The accumulation of static charges can result in fog patterns in photographic emulsions, various coating imperfections such as mottle patterns and repellency spots, dirt and dust attraction which may result in the formation of "pinholes" in processed films, and a variety of handling and conveyance problems.

To overcome the problem of accumulation of static charges it is conventional practice to provide an antistatic layer in photographic elements. Many antistatic agents have been utilized for this purpose. For example, an antistatic layer comprising an alkali metal salt of a copolymer of styrene and styrylundecanoic acid is disclosed in U.S. Pat. No. 3,033,679. Photographic films having a metal halide, such as sodium chloride or potassium chloride, as the conducting material, in a hardened polyvinyl alcohol binder are described in U.S. Pat. No. 3,437,484. In U.S. Pat. No. 3,525,621, the antistatic layer is comprised of colloidal silica and an organic antistatic agent, such as an alkali metal salt of an alkylaryl polyether sulfonate, an alkali metal salt of an arylsulfonic acid, or an alkali metal salt of a polymeric carboxylic acid. An antistatic layer comprised of an anionic film forming polyelectrolyte, colloidal silica and a polyalkylene oxide is disclosed in U.S. Pat. No. 3,630,740. In U.S. Pat. No. 3,681,070, an antistatic layer is described in which the antistatic agent is a copolymer of styrene and styrene sulfonic acid. U.S. Pat. No. 4,542,095 describes antistatic compositions comprising a binder, a nonionic surface-active polymer having polymerized alkylene oxide monomers and an alkali metal salt. In U.S. Pat. No. 4,916,011, an antistatic layer comprising a styrene sulfonate-maleic acid copolymer, a latex binder, and an alkyl-substituted trifunctional aziridine crosslinking agent is disclosed.

It is known to prepare an antistatic layer from a composition comprising a vanadium pentoxide colloidal gel as described, for example, in U.S. Pat. No. 4,203,769. Antistatic layers containing vanadium pentoxide provide excellent protection against static and are highly advantageous in that they have excellent transparency and their performance is not significantly dependent on humidity. The excellent performance of these antistatic layers results from the particular morphology of this material. The colloidal vanadium pentoxide gel consists of entangled, high aspect ratio, flat ribbons about 50-100 angstroms wide, about 10 angstroms thick and about 1000-10000 angstroms long. Low surface resistivities can be obtained with very low vanadium pentoxide coverages as a result of this high aspect ratio morphology.

Typically, the vanadium pentoxide is coated in a polymeric binder to improve adhesion to adjacent layers and to improve the durability of the antistatic layer. Polyesterionomer dispersions, which are preferred binders because they exhibit excellent film-forming properties and compatibility with vanadium pentoxide, have recently been disclosed for use in aqueous-based, vanadium pentoxide-containing antistatic coating formulations. For example, an element comprising a support, at least one imaging layer, and an antistatic layer comprising vanadium pentoxide in a polyesterionomer binder containing carboxyl groups, alkali metal carboxylate groups, sulfonic acid groups, or alkali metal sulfonate groups is described in U.S. Pat. No. 5,360,706. An imaging element for use in electrostatography containing an electrically-conductive layer comprising vanadium pentoxide dispersed in a polymer binder such as a polyesterionomer dispersion is described in U.S. Pat. No. 5,380,584. Antistatic layers containing vanadium pentoxide in sulfopolymer binders, including sulfopolymers are described in U.S. Pat. Nos. 5,203,884, 5,322,761, 5,372,985, 5,407,603, 5,424,269, 5,427,835, 5,439,785, and 5,468,498.

It is known to overcoat a vanadium pentoxide antistatic layer with a hydrophobic, protective overcoat or barrier layer to prevent the dissolution of the antistatic material in film processing solutions which would otherwise result in a diminution of the antistatic properties. Such barrier layers are described in U.S. Pat. Nos. 5,006,451 and 5,221,598, for example. However, the need to overcoat a vanadium pentoxide layer with a barrier layer has several potential disadvantages. These include the following:

(1) An additional layer must be coated and dried. This increases both manufacturing complexity and cost.

(2) In some critical applications it may be desirable to have the antistatic layer serve as the surface layer since there may be some loss in the effectiveness of the antistatic properties when the conductive layer is buried below an electrically-insulating, barrier layer.

(3) When a protective overcoat for the antistatic layer is desired to provide other properties such as friction control, abrasion resistance, ferotyping and blocking resistance, etc., the choice of materials for the protective overcoat is limited by the need for the layer to also serve as a barrier layer.

(4) It may be desirable to overcoat the antistatic layer with a water (or film processing solution) permeable, hydrophilic layer such as a curl control layer or pelloid layer. However, such permeable layers can not prevent the dissolution of the vanadium pentoxide.

As mentioned hereinabove, it is known from U.S. Pat. No. 5,360,706 to form an antistatic layer of an imaging element by dispersing electrically-conductive colloidal vanadium pentoxide in a polyesterionomer binder. As described in the '706 patent, use of a polyesterionomer binder provides improved coating solution stability and enhanced interlayer adhesion. However, a hydrophobic protective overcoat is required to obtain process-surviving antistatic protection.

It is known from U.S. Pat. No. 5,427,835 to form antistatic layers from an aqueous-based mixture comprising colloidal vanadium pentoxide and a dispersed sulfonated polymer but such mixtures lack the degree of process-surviving capability desired in imaging elements.

It is known from U.S. Pat. No. 5,096,975 to form an antistatic layer of an imaging element from a combination of a copolymer of vinylbenzene sulfonic acid and a methoxy-alkylmelamine crosslinking agent. As described in the '975 patent, this combination provides process-surviving anti-

static protection. However, the conductive properties are humidity dependent.

For many imaging elements, and especially photographic films and papers, it is important that the electrically-conductive properties be essentially independent of humidity. Thus, for example, photothermographic elements are typically developed by heating in a high temperature processing chamber in which relative humidity is very low and a layer which is electrically-conductive only under conditions of high relative humidity is entirely unsatisfactory. Equally important for many imaging elements is the requirement that the electrical conductivity be process-surviving. Thus, for example, the electrically-conductive layer must not dissolve in a developing solution or other solutions employed in processing the imaging element. If the electrically-conductive layer is an outermost layer, it is also highly desirable that it resist softening or becoming tacky as a result of contact with processing baths as a soft and tacky surface is easily damaged and prone to dirt pickup in processing equipment.

It is toward the objective of providing an improved electrically-conductive layer for imaging elements whose conductivity is both process-surviving and humidity-independent that the present invention is directed.

#### SUMMARY OF THE INVENTION

In accordance with this invention, an imaging element for use in an image-forming process is comprised of a support, an image-forming layer and an electrically-conductive layer whose electrical conductivity is process-surviving and essentially independent of humidity. The electrically-conductive layer is comprised of a vanadium pentoxide colloidal gel, a polyesterionomer binder and a methoxyalkylmelamine.

In a particular embodiment, the invention is directed to a substrate for use as a component of an imaging element, the substrate comprising a support having thereon an electrically-conductive layer comprised of a vanadium pentoxide colloidal gel, a polyesterionomer binder and a methoxyalkylmelamine.

In a further particular embodiment, the invention is directed to a coating composition that is useful for forming an electrically-conductive layer of an imaging element, the coating composition comprising a vanadium pentoxide colloidal gel, a polyesterionomer binder and a methoxyalkylmelamine.

#### DETAILED DESCRIPTION OF THE INVENTION

The imaging elements of this invention can be of many different types depending on the particular use for which they are intended. Such elements include, for example, photographic, electrostatographic, photothermographic, migration, electrothermographic, dielectric recording and thermal-dye-transfer imaging elements.

Details with respect to the composition and function of a wide variety of different imaging elements are provided in U.S. Pat. No. 5,340,676 and references described therein. The present invention can be effectively employed in conjunction with any of the imaging elements described in the '676 patent.

Photographic elements represent an important class of imaging elements within the scope of the present invention. In such elements, the electrically-conductive layer may be

applied as a subbing layer, as an intermediate layer, or as the outermost layer on the sensitized emulsion side of the support, on the side of the support opposite the emulsion, or on both sides of the support.

5 The support material utilized in this invention can be comprised of various polymeric films, paper, glass, and the like, but, polyester film support, which is well known in the art, is preferred. The thickness of the support is not critical. Support thicknesses of 2 to 10 mil (0.05 to 0.25 millimeters) can be employed, for example, with very satisfactory results. 10 The support material typically employs an - undercoat or primer layer between the antistatic layer and the polyester support. Such undercoat layers are well known in the art and comprise, for example, a vinylidene chloride/methyl acrylate/itaconic acid terpolymer or vinylidene chloride/acrylonitrile/acrylic acid terpolymer.

15 The antistatic layer of this invention comprises a colloidal gel of vanadium pentoxide as the conductive material. The use of vanadium pentoxide in antistatic layers is described in Guestaux, U.S. Pat. No. 4,203,769. The antistatic layer is prepared by coating an aqueous colloidal solution of vanadium pentoxide, a water-dispersible polyesterionomer binder, and a methoxyalkylmelamine. Preferably, the vanadium pentoxide is doped with silver. Typically the dried coating weight of the vanadium pentoxide antistatic material is about 0.5 to about 50 mg/m<sup>2</sup>. The ratio of the total weight of the polyesterionomer binder plus methoxyalkylmelamine to the vanadium pentoxide antistatic material is at least 25:1 to insure an impermeable coating and less than 200:1 to yield useful electrical resistivity values before and after film processing (i.e., electrical resistivity less than or equal to 5×10<sup>11</sup> ohms per square).

20 Methoxyalkylmelamines are well known crosslinking agents for polymers containing hydroxyl, carboxyl, and amide groups. U.S. Pat. Nos. 5,096,975 and 5,198,499, for example, describe electrically-conductive copolymers of vinylbenzene sulfonic acid and a hydroxyl-containing monomer crosslinked with a methoxyalkylmelamine. In the present invention it is not clear whether the improved resistance to permeation by film processing solutions is due to reaction of the methoxyalkylmelamine with the polyesterionomer binder, self-condensation of the methoxyalkylmelamine, or some combination of these two reactions. In the present invention, the weight ratio of polyesterionomer binder to methoxyalkylmelamine is preferably about 4:1 to about 48:1 and more preferably about 4:1 to about 24:1. Use of too little methoxyalkylmelamine deleteriously affects the impermeability of the antistatic layer. However, if an excessive amount of the methoxyalkylmelamine is used it may remain unreacted in the electrically-conductive layer, thus 25 acting as a plasticizer and decreasing the water and chemical resistance of the coating. An acid catalyst such as a mineral acid, an aromatic sulfonic acid, phosphoric acid, alkyl phosphoric acid, etc. may be added to the coating formulation to improve the rate of curing. Preferably the acid catalyst is an aryl sulfonic acid such as p-toluene sulfonic acid. The acid catalyst may be present in an amount of 0.1 to 2% of the total weight of the methoxyalkylmelamine compound.

30 Any methoxyalkylmelamine may be employed in this invention such as, for example, those multifunctional methoxyalkylmelamines having at least 2 and preferably 3 to 6 methoxyalkyl groups, such as hexamethoxymethylmelamine, trimethoxymethylmelamine, hexamethoxyethylmelamine, tetramethoxyethylmelamine, hexamethoxypropylmelamine, pentamethoxypropylmelamine, trimethoxybutylmelamine, and the like. It is preferred that hexamethoxymethylmelamine be employed.

The term "polyesterionomer" refers to polyesters that contain at least one ionic moiety. Such ionic moieties function to make the polymer water dispersible. These polyesters are prepared by reacting one or more dicarboxylic acids or their functional equivalents such as anhydrides, diesters, or diacid halides with one or more diols in melt phase polycondensation techniques well known in the art (see for example, U.S. Pat. Nos. 3,018,272, 3,929,489, 4,307,174, 4,419,437). Examples of this class of polymers include, for example, Eastman AQ® polyesterionomers, manufactured by Eastman Chemical Co.

Typically the ionic moiety is provided by some of the dicarboxylic acid repeat units, the remainder of the dicarboxylic acid repeat units are nonionic in nature. Such ionic moieties can be anionic or cationic, but, for the purpose of the present invention the ionic group must be anionic in nature to prevent flocculation of the colloidal vanadium pentoxide antistat. Preferably the ionic dicarboxylic acid contains a sulfonic acid group or its metal salt. Examples include the sodium, lithium, or potassium salt of sulfoterephthalic acid, sulfonaphthalene dicarboxylic acid, sulfophthalic acid, and sulfoisophthalic acid or their functionally equivalent anhydride, diester, or diacid halide. Most preferably the ionic dicarboxylic acid repeat unit is provided by 5-sodiosulfoisophthalic acid or dimethyl 5-sodiosulfoisophthalate. The nonionic dicarboxylic acid repeat units are provided by dicarboxylic acids or their functional equivalents represented by the formula:



where R is an aromatic or aliphatic hydrocarbon or contains both aromatic and aliphatic hydrocarbons. Exemplary compounds include isophthalic acid, terephthalic acid, succinic acid, adipic acid, and others.

Suitable diols are represented by the formula: HO—R—OH, where R is aromatic or aliphatic or contains both aromatic and aliphatic hydrocarbons. Preferably the diol includes one or more of the following: ethylene glycol, diethylene glycol, or 1,4-cyclohexanedimethanol.

The polyesterionomer binders of the invention preferably comprise from about 1 to about 25 mol %, based on the total moles of dicarboxylic acid repeat units, of the ionic dicarboxylic acid repeat units. Preferably the polyesterionomers have a glass transition temperature ( $T_g$ ) of about 0° C. to 100° C. More preferably, the  $T_g$  is about 20° C. to about -80° C.

The use of polyesterionomer dispersions in aqueous coating formulations, for example, inks, has been reported. U.S. Pat. Nos. 4,883,714, 4,847,316, 4,738,785 and 4,704,309 describe aqueous printing inks using polyesterionomers as a pigment carrier or binder.

U.S. Pat. No. 4,307,174 describes water-dispersible polyester adhesives for photographic materials. U.S. Pat. No. 4,419,437 describes polyesterionomers useful to disperse particulate pigments in, for example, image-forming compositions such as for lithographic plates.

Polyesterionomers have been reported as priming layers on photographic film supports. U.S. Pat. No. 4,883,706 describes a composite polyester film comprising a coating, e.g. a coextruded layer, of a sulfonated polyester adhesion primer on one or both sides of a semicrystalline polyester film substrate. U.S. Pat. No. 4,394,442 describes a subbing layer comprising a water-dispersible polyesterionomer applied to an energy-treated, biaxially-oriented polyester film base. U.S. Pat. No. 4,478,907 discloses a subbing layer

for polyester film support comprising a water-dispersible polyesterionomer with a  $T_g$  of at least 50° C. derived from ethylene glycol and a mixture of isophthalic acid, a salt of sulfoisophthalic acid, terephthalic acid, and an aromatic dicarboxylic acid. Research Disclosure 241008 describes a dispersion suitable for subbing polyester film support comprised of a polyester containing repeat units derived from a polyhydroxy compound and a mixture of terephthalic acid, isophthalic acid, and a salt of sulfoisophthalic acid in which at least one of the polyhydroxy compounds or diacids contain a  $\text{CCl}_3$  group. An antistatic layer for a photographic film support consisting essentially of a blockcopolyetherester of dibasic carboxylic acid(s) esterified with ethylene glycol that may contain a small amount of sulfo groups in salt form is described in European Patent Application 247648. However, the polyester was not reported to be a binder for an antistatic agent.

U.S. Pat. No. 5,439,785 describes a photographic element comprising antistatic layers of vanadium pentoxide, a sulfopolymer which includes sulfopolyesters, and an adhesion promoting compound. Epoxy silanes are disclosed as the adhesion promoting compound. Examples are described for antistatic layers containing vanadium pentoxide and a sulfopolyester with and without the adhesion promoting epoxy silane compound. The layers reportedly provide antistatic protection after film processing.

The antistatic coating of the invention may be applied onto the film support using coating methods well known in the art such as hopper coating, skim pan/air knife coating, 30 gravure coating, and others. In the drying and curing of the antistatic layer, temperatures of from about 25° C. to about 200° C. may be employed. Preferably a temperature of from about 80° C. to about 140° C. for approximately 3 to 10 minutes is employed.

In addition to the vanadium pentoxide, polyesterionomer binder, methoxyalkylmelamine, and acid catalyst, other ingredients well known in the photographic art may be added to the antistatic coating composition. These include, anionic and nonionic surfactants and wetting aids, matte particles, and lubricants. The antistatic layer of this invention may serve as the outermost layer of an imaging element or it can be overcoated with various types of protective overcoats (for example, cellulose esters, polyurethanes, polyesters, acrylate and/or methacrylate containing interpolymers), gelatin subbing layers, silver halide emulsions, and gelatin curl control layers.

In a particularly preferred embodiment, the imaging elements of this invention are photographic elements, such as photographic films, photographic papers or photographic glass plates, in which the image-forming layer is a radiation-sensitive silver halide emulsion layer. Such emulsion layers typically comprise a film-forming hydrophilic colloid. The most commonly used of these is gelatin and gelatin is a particularly preferred material for use in this invention. Useful gelatins include alkali-treated gelatin (cattle bone or hide gelatin), acid-treated gelatin (pigskin gelatin) and gelatin derivatives such as acetylated gelatin, phthalated gelatin and the like. Other hydrophilic colloids that can be utilized alone or in combination with gelatin include dextran, gum arabic, zein, casein, pectin, collagen derivatives, collodion, agar-agar, arrowroot, albumin, and the like. Still other useful hydrophilic colloids are water-soluble polyvinyl compounds such as polyvinyl alcohol, polyacrylamide, poly(vinylpyrrolidone), and the like.

The photographic elements of the present invention can be simple black-and-white or monochrome elements comprising a support bearing a layer of light-sensitive silver

halide emulsion or they can be multilayer and/or multicolor elements.

Color photographic elements of this invention typically contain dye image-forming units sensitive to each of the three primary regions of the spectrum. Each unit can be comprised of a single silver halide emulsion layer or of multiple emulsion layers sensitive to a given region of the spectrum. The layers of the element, including the layers of the image-forming units, can be arranged in various orders as is well known in the art.

A preferred photographic element according to this invention comprises a support bearing at least one blue-sensitive silver halide emulsion layer having associated therewith a yellow image dye-providing material, at least one green-sensitive silver halide emulsion layer having associated therewith a magenta image dye-providing material and at least one red-sensitive silver halide emulsion layer having associated therewith a cyan image dye-providing material.

In addition to emulsion layers, the elements of the present invention can contain auxiliary layers conventional in photographic elements, such as overcoat layers, spacer layers, filter layers, interlayers, antihalation layers, pH lowering layers (sometimes referred to as acid layers and neutralizing layers), timing layers, opaque reflecting layers, opaque light-absorbing layers and the like. The support can be any suitable support used with photographic elements. Typical supports include polymeric films, paper (including polymer-coated paper), glass and the like. Details regarding supports and other layers of the photographic elements of this invention are contained in *Research Disclosure*, Item 36544, September, 1994.

The light-sensitive silver halide emulsions employed in the photographic elements of this invention can include coarse, regular or fine grain silver halide crystals or mixtures thereof and can be comprised of such silver halides as silver chloride, silver bromide, silver bromoiodide, silver chlorobromide, silver chloroiodide, silver chlorobromoiodide, and mixtures thereof. The emulsions can be, for example, tabular grain light-sensitive silver halide emulsions. The emulsions can be negative-working or direct positive emulsions. They can form latent images predominantly on the surface of the silver halide grains or in the interior of the silver halide grains. They can be chemically and spectrally sensitized in accordance with usual practices. The emulsions typically will be gelatin emulsions although other hydrophilic colloids can be used in accordance with usual practice. Details regarding the silver halide emulsions are contained in *Research Disclosure*, Item 36544, September, 1994, and the references listed therein.

The photographic silver halide emulsions utilized in this invention can contain other addenda conventional in the photographic art. Useful addenda are described, for example, in *Research Disclosure*, Item 36544, September, 1994. Useful addenda include spectral sensitizing dyes, desensitizers, antifoggants, masking couplers, DIR couplers, DIR compounds, antistain agents, image dye stabilizers, absorbing materials such as filter dyes and UV absorbers, light-scattering materials, coating aids, plasticizers and lubricants, and the like.

Depending upon the dye-image-providing material employed in the photographic element, it can be incorporated in the silver halide emulsion layer or in a separate layer associated with the emulsion layer. The dye-image-providing material can be any of a number known in the art, such as dye-forming couplers, bleachable dyes, dye developers and redox dye-releasers, and the particular one employed will depend on the nature of the element, and the type of image desired.

Dye image-providing materials employed with conventional color materials designed for processing with separate solutions are preferably dye-forming couplers; i.e., compounds which couple with oxidized developing agent to form a dye. Preferred couplers which form cyan dye images are phenols and naphthols. Preferred couplers which form magenta dye images are pyrazolones and pyrazolotriazoles. Preferred couplers which form yellow dye images are benzoylacetanilides and pivalylacetanilides.

Although each of the individual components contained in the antistatic layer of this invention is known for use in imaging elements it was unexpected that such a combination of components would provide an antistatic coating composition that has excellent solution stability and freedom from flocculation of the vanadium pentoxide as well as the ability to provide a dried layer whose antistatic properties survive even the most demanding film processing conditions. The invention is further illustrated by the following examples of its practice.

#### EXAMPLES 1-10

Solution A was prepared by adding 235 grams of a 25.5 weight % dispersion of a polyesterionomer having a  $T_g$  of 55° C. (this polyesterionomer is available from Eastman Chemical Co. in solid pellet form as EASTMAN AQ@ 55S), 60 grams of hexamethoxymethylmelamine (available as Cymel 303 Resin, Cytec Industries, Inc.), and 10 grams of a 10% solution of Olin 10 G nonionic surfactant to 165 grams of deionized water. This solution was mixed at room temperature for several hours and then used in the following coating formulations.

Solution 1 was prepared by mixing 3.75 grams of a 0.57% silver-doped vanadium pentoxide colloidal dispersion, 35.8 grams of deionized water, 5 grams of the 25.5% polyesterionomer dispersion, 0.07 grams of 6.7% Triton X-100 surfactant (available from Rohm and Haas Company), 3.34 grams of Solution A, and 2 grams of 1% p-toluene sulfonic acid.

Solution 2 was prepared by mixing 3.75 grams of a 0.57% silver-doped vanadium pentoxide colloidal dispersion, 35.8 grams of deionized water, 6.48 grams of the 25.5% polyesterionomer dispersion, 0.07 grams of 6.7% Triton X-100 surfactant (available from Rohm and Haas Company), 1.86 grams of Solution A, and 2 grams of 1% p-toluene sulfonic acid.

Solution 3 was prepared by mixing 3.75 grams of a 0.57% silver-doped vanadium pentoxide colloidal dispersion, 42.1 grams of deionized water, 1.25 grams of the 25.5% polyesterionomer dispersion, 0.07 grams of 6.7% Triton X-100 surfactant (available from Rohm and Haas Company), 0.835 grams of Solution A, and 2 grams of 1% p-toluene sulfonic acid.

Solution 4 was prepared by mixing 3.75 grams of a 0.57% silver-doped vanadium pentoxide colloidal dispersion, 40 grams of deionized water, 2.5 grams of the 25.5% polyesterionomer dispersion, 0.07 grams of 6.7% Triton X-100 surfactant (available from Rohm and Haas Company), 1.67 grams of Solution A, and 2 grams of 1% p-toluene sulfonic acid.

Solution 5 was prepared by mixing 3.75 grams of a 0.57% silver-doped vanadium pentoxide colloidal dispersion, 40.0 grams of deionized water, 3.24 grams of the 25.5% polyesterionomer dispersion, 0.07 grams of 6.7% Triton X-100 surfactant (available from Rohm and Haas Company), 0.93 grams of Solution A, and 2 grams of 1% p-toluene sulfonic acid.

Solution 6 was prepared by mixing 3.75 grams of a 0.57% silver-doped vanadium pentoxide colloidal dispersion, 35.8 grams of deionized water, 6.95 grams of the 25.5% polyesterionomer dispersion, 0.07 grams of 6.7% Triton X-100 surfactant (available from Rohm and Haas Company), 1.40 grams of Solution A, and 2 grams of 1% p-toluene sulfonic acid.

Solution 7 was prepared by mixing 3.75 grams of a 0.57% silver-doped vanadium pentoxide colloidal dispersion, 35.8 grams of deionized water, 7.41 grams of the 25.5% polyesterionomer dispersion, 0.07 grams of 6.7% Triton X-100 surfactant (available from Rohm and Haas Company), 0.93 grams of Solution A, and 2 grams of 1% p-toluene sulfonic acid.

Solution 8 was prepared by mixing 3.75 grams of a 0.57% silver-doped vanadium pentoxide colloidal dispersion, 35.8 grams of deionized water, 7.64 grams of the 25.5% polyesterionomer dispersion, 0.07 grams of 6.7% Triton X-100 surfactant (available from Rohm and Haas Company), 0.70 grams of Solution A, and 2 grams of 1% p-toluene sulfonic acid.

Solution 9 was prepared by mixing 3.75 grams of a 0.57% silver-doped vanadium pentoxide colloidal dispersion, 35.8 grams of deionized water, 7.88 grams of the 25.5% polyesterionomer dispersion, 0.07 grams of 6.7% Triton X-100 surfactant (available from Rohm and Haas Company), 0.47 grams of Solution A, and 2 grams of 1% p-toluene sulfonic acid.

Solution 10 was prepared by mixing 3.75 grams of a 0.57% silver-doped vanadium pentoxide colloidal dispersion, 35.8 grams of deionized water, 7.99 grams of the

5 polyesterionomer dispersion, and 0.15 grams of 6.7% Triton X-100 surfactant (available from Rohm and Haas Company). This solution represents a comparative formulation analogous to that described in U.S. Pat. No. 5,439,785 to prepare Example 1, film 5. This film was reported to provide antistatic properties after processing in standard KODAK PROCESS C41 film processing.

The above solutions 1 to 12 were coated onto a polyethylene terephthalate support that had been previously coated with a vinylidene chloride-containing terpolymer latex subbing layer. Solutions 1 through 11 were applied at a wet coverage of 24 ml/m<sup>2</sup> and solution 12 was applied at a wet coverage of 6 ml/m<sup>2</sup>. All of the coatings were dried at 100° C. for 3 minutes. The surface resistivity for the coatings at 20% RH was measured using a two-point probe before and after processing in KODAK ULTRATEC processing chemistry. This is a high pH, high temperature film development process that represents a severe test for antistatic performance survivability. The results for the coatings are reported in Table 1.

The results show that coatings of the invention which contain the polyesterionomer, hexamethoxymethylmelamine and vanadium pentoxide provide excellent resistivity values before and after processing. In addition, all of the coating solutions of the invention have excellent stability and form highly transparent films. Comparative coatings that do not contain the hexamethoxymethylmelamine do not provide effective antistatic performance after processing in the KODAK ULTRATEC processing chemistry.

TABLE 1

| Coating       | Solution | Polyesterionomer/<br>Hexamethoxymethylmelamine<br>Weight Ratio | Surface Resistivity<br>Before Processing,<br>ohms per square | Surface Resistivity<br>After Processing,<br>ohms per square |
|---------------|----------|----------------------------------------------------------------|--------------------------------------------------------------|-------------------------------------------------------------|
| Example 1     | 1        | 4/1                                                            | $3.1 \times 10^7$                                            | $8.0 \times 10^7$                                           |
| Example 2     | 2        | 8/1                                                            | $4.0 \times 10^7$                                            | $8.0 \times 10^7$                                           |
| Example 3     | 3        | 4/1                                                            | $2.5 \times 10^8$                                            | $7.9 \times 10^{10}$                                        |
| Example 4     | 4        | 4/1                                                            | $3.2 \times 10^8$                                            | $6.3 \times 10^9$                                           |
| Example 5     | 5        | 8/1                                                            | $1.0 \times 10^8$                                            | $1.0 \times 10^9$                                           |
| Example 6     | 6        | 12/1                                                           | $2.5 \times 10^8$                                            | $4.0 \times 10^8$                                           |
| Example 7     | 7        | 16/1                                                           | $2.5 \times 10^8$                                            | $3.1 \times 10^8$                                           |
| Example 8     | 8        | 24/1                                                           | $4.0 \times 10^8$                                            | $5.0 \times 10^8$                                           |
| Example 9     | 9        | 32/1                                                           | $4.0 \times 10^8$                                            | $3.1 \times 10^9$                                           |
| Example 10    | 10       | 48/1                                                           | $4.0 \times 10^8$                                            | $3.1 \times 10^{10}$                                        |
| Comparative 1 | 11       | —                                                              | $4.0 \times 10^7$                                            | $>1 \times 10^{13}$                                         |
| Comparative 2 | 12       | —                                                              | $4.0 \times 10^8$                                            | $>1 \times 10^{13}$                                         |

50 25.5% polyesterionomer dispersion, 0.07 grams of 6.7% Triton X-100 surfactant (available from Rohm and Haas Company), 0.35 grams of Solution A, and 2 grams of 1% p-toluene sulfonic acid.

Solution 11 was prepared by mixing 3.75 grams of a 0.57% silver-doped vanadium pentoxide colloidal dispersion, 37.8 grams of deionized water, 8.34 grams of the 25.5% polyesterionomer dispersion, and 0.07 grams of 6.7% Triton X-100 surfactant (available from Rohm and Haas Company). This solution represents a comparative formulation that does not contain the hexamethoxymethylmelamine, but has the polyesterionomer binder and the vanadium pentoxide antistatic material at a weight ratio of 100:1.

Solution 12 was prepared by mixing 2.2 grams of a 0.57% silver-doped vanadium pentoxide colloidal dispersion, 45.7 grams of deionized water, 1.96 grams of the 25.5% poly-

55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765

## 11

The invention has been described in detail with particular reference to certain preferred embodiments thereof, but it will be understood that variations and modifications can be effected within the spirit and scope of the invention.

We claim:

1. An imaging element for use in an image-forming process; said imaging element comprising a support, an image-forming layer and an electrically-conductive layer; said electrically-conductive layer comprising a vanadium pentoxide colloidal gel, a polyesterionomer binder and a methoxyalkylmelamine. 10
2. An imaging element as claimed in claim 1, wherein said support is a polyester film.
3. An imaging element as claimed in claim 1, wherein said vanadium pentoxide is doped with silver.
4. An imaging element as claimed in claim 1, wherein the dried coating weight of said electrically-conductive layer is about 0.5 to about 50 mg/m<sup>2</sup>.
5. An imaging element as claimed in claim 1, wherein the ratio of the total weight of polyesterionomer binder plus methoxyalkylmelamine to vanadium pentoxide is at least 25:1 and less than 200:1. 20
6. An imaging element as claimed in claim 1, wherein the weight ratio of polyesterionomer binder to methoxyalkylmelamine is from about 4:1 to about 48:1.
7. An imaging element as claimed in claim 1, wherein the

5

15

25

## 12

weight ratio of polyesterionomer binder to methoxyalkylmelamine is from about 4:1 to about 24:1.

8. An imaging element as claimed in claim 1, wherein said methoxyalkylmelamine has 3 to 6 methoxyalkyl groups.
9. An imaging element as claimed in claim 1, wherein said methoxyalkylmelamine is hexamethoxymethylmelamine.
10. An imaging element as claimed in claim 1, wherein said polyesterionomer has a glass transition temperature of about 20° C. to about 80° C.
11. An imaging element as claimed in claim 1, wherein said element is a photographic element.
12. An imaging element as claimed in claim 1, wherein said element is a photothermographic element.
13. An imaging element as claimed in claim 1, wherein said image-forming layer is a silver halide emulsion layer.
14. A substrate that is useful as a component of an imaging element, said substrate comprising a support having thereon an electrically-conductive layer; said electrically-conductive layer comprising a vanadium pentoxide colloidal gel, a polyesterionomer binder and a methoxyalkylmelamine.
15. A coating composition that is useful for forming an electrically-conductive layer of an imaging element; said coating composition comprising a vanadium pentoxide colloidal gel, a polyesterionomer binder and a methoxyalkylmelamine.

\* \* \* \* \*